

# UNITED STATES PATENT OFFICE.

OTTO FISCHER, OF STUTTGART, GERMANY, ASSIGNEE TO FIRM OF ROBERT BOSCH, OF STUTTGART, GERMANY.

## SHAPING FIBER ARTICLES.

1,275,888.

Specification of Letters Patent. Patented Aug. 13, 1918.

No Drawing.

Application filed January 6, 1913. Serial No. 740,554.

*To all whom it may concern:*

Be it known that I, OTTO FISCHER, a subject of the Emperor of Germany, residing at Stuttgart, Spittastrasse 8, Germany, have 5 invented certain new and useful Improvements in Shaping Fiber Articles; and I do hereby declare the following to be a full, clear, and exact description of the invention, such as will enable others skilled in the art to 10 which it appertains to make and use the same.

The dense brittle fibrous material now widely used in the electrical arts for purposes of insulation, particularly in the form 15 of insulating tubes for electric conducting cables, and known to the trade as "fiber" or "red fiber" is of such a character that, in its ordinary commercial condition, it cannot be bent without breaking; so that when it 20 has been desired to use a bent tube, as is frequently the case, no method has been known whereby the finished tubes could be bent.

The subject-matter of the present application 25 is based upon the discovery that objects of "fiber" can be bent very considerably if they are first caused to swell, with increase of pliability, through the agency of moisture within the pores of the material; 30 and that articles so treated will retain the bend imparted to them and take a permanent set in the new shape if they are restrained by mechanical means in the new shape until the agency which has caused the 35 material to swell has been withdrawn.

I have found that the requisite swelling and increase of pliability can be effected by 40 means of the moisture content of the material itself, which is quite considerable, if heat is applied to expand the contained moisture, as by heating the unbent fiber articles over a flame, care being taken that the material is not burned. It is likewise possible to produce the desired swelling of the 45 material by the application of moisture without the application of heat, as by soaking the material in water, since the material is extremely hygroscopic. The method succeeds best, however, if the parts to be bent 50 are immersed in a liquid which has been heated to the desired temperature.

After the material has been so treated it may be bent to the desired shape, and should then be held by mechanical means in that 55 shape until it has been cooled or dried, or

cooled and dried, as the case may be. As soon as the normal condition of temperature and dryness has been reached, the article assumes again its original stiffness and brittleness, and the bent object will, if properly 60 treated, retain without change the bent shape imparted to it.

By this method I have been able, for example, to bend without difficulty and give a permanent set to a "fiber" tube of one inch 65 external diameter, the bend taking the form of a right angle, it being understood that during the bending operation suitable precautions are taken to avoid flattening the tube at the place of bending. Such a bent 70 article may be installed in usual places, there being no material reduction of its insulating properties.

After the conclusion of the bending operation it is possible, and even preferable, to 75 prevent the re-absorption of moisture by impregnating the article with a moisture-excluding material such as paraffin. This may be accomplished by laying the shaped and stiff article in melted paraffin, which 80 then fills the pores and hardens, when the article is removed from the bath and cooled.

In those cases in which the bent parts are prevented by the manner of their ultimate employment as, for instance, by confinement 85 in the places where they are installed, from coming back into the original unbent position, the method requires no further enlargement. In many cases, however, as when a "fiber" tube is used to protect elec- 90

tric conducting cables which are to be freely suspended, the treated and bent objects must be protected against the re-absorption of moisture from the air, since otherwise they would soon return to their original unbent 95 shape and, moreover, they are not always sufficiently insulating after undergoing the described treatment. For this purpose the bent objects may be provided with a coating of lacquer or other moisture-excluding material, and as long as the coating of lacquer 100 remains in good condition the bent object will retain the shape imparted to it.

The bending and protecting steps in the process hereinbefore described may, with 105 advantage, be effected simultaneously by immersing the material in a heated bath of melted paraffin or other moisture-repelling material until it has acquired the requisite swelling and increase of pliability, then 110

bending the article and securing it in the bent shape, and then allowing the absorbed paraffin to cool and solidify so as to fill the pores and prevent subsequent absorption of moisture.

Having thus described my invention what I claim is:

1. The method of treating tubes composed of dense brittle fibrous insulating material such as that known as "fiber" to shape them, which consists in immersing a portion of the tube in a heated bath of a waxy material such as paraffin to soften it and make the material of the tube pliable then bending the tube to the desired shape while it is in the softened pliable condition and while impregnated with the material of the bath, and maintaining the tube in the new shape until, as a result of drying and cooling, it stiffens and sets with the pores thereof containing the material of the bath in a hardened form; substantially as described.

2. The method of treating articles composed of dense brittle fibrous insulating material commercially known as "fiber" to shape them and to cause them to retain the new shape, which consists in causing them to swell with an increase of pliability by immersion in a heated bath, bending the

swelled and pliable article to the desired shape, maintaining it in that shape while withdrawing the softening agency until the article stiffens and sets in the new shape, and applying a water-proofing material to the article to prevent the subsequent absorption of moisture thereby; substantially as described.

3. The method of treating articles made of fibrous insulating material which is dense and brittle when hard and which is commercially known as "fiber", which consists in making a rigid article from the material, causing the article to swell and become pliable by immersion in a heated bath, bending the swelled and pliable article to the desired shape, maintaining it in that shape while withdrawing the softening agency until the article stiffens and sets in the new shape and applying a waterproofing material to the article to prevent subsequent absorption of moisture thereby; substantially as described.

In testimony whereof I affix my signature, in presence of two witnesses.

OTTO FISCHER.

Witnesses:

PAUL WOLFORT,  
HERMANN SCHNEIDER.